

## UNITED STATES PATENT OFFICE

2,314,380

## PHOTOGRAPHIC REVERSAL PROCESS

James R. Alburger, Merion, Pa., assignor to Radio Corporation of America, a corporation of Delaware

No Drawing. Application May 31, 1940.  
Serial No. 338,051

7 Claims. (Cl. 95—88)

This invention relates to a photographic reversal process particularly adapted for use with motion picture film and more specifically adapted for use with ordinary positive types of film for taking the original picture and producing the reversal print.

In the practice of the production of positive pictures by the reversal process, as customarily applied, for example, to the production of 16 mm. and 8 mm. motion pictures, a specially coated type of film is used for the reason that the reversal processes heretofore employed failed to give either clear whites or proper gradation when applied to ordinary types of film.

In the present process it is possible to use ordinary positive motion picture film for the original exposure and to produce perfectly satisfactory positives therefrom and with this positive film showing an effective speed of from 10 to 30 times that which it ordinarily shows when developed according to the customary methods. The improved process further prevents to a large extent the reticulation which often occurs in the application of reversal processes.

In the performance of my improved process I use a hardening developer of the general type described and claimed in my Patent No. 2,199,904, thereby preventing reticulation, and by overdeveloping somewhat and partially dissolving the silver salts in the image I secure the proper residual amount of silver for the production of the positive image.

One object of the invention is to provide an improved photographic reversal process.

Another object of the invention is to provide a photographic reversal process which permits the use of positive film.

Another object of the invention is to provide a photographic reversal process which greatly increases the effective speed of film used.

Other and incidental objects of the invention will be apparent to this skilled in the art from a reading of the following specification.

In the preferred manner of performing my process, I use an ordinary positive motion picture film. One type of such film which is appropriate for the purpose is that known commercially as EK 1301, although any equivalent positive film stock may be used as desired, for example, the type known as Dupont Micro-Pan is quite satisfactory.

In the exposure of the film a speed rating of from 10 to 30 times the normal speed rating is given to the film. For example, the EK 1301 film is normally rated at Weston 1, while for

15 pictures of average subject matter a rating of 16 may be used for this film when developed according to my process, and for scenes having considerable sky or water in them a rating as high as 32 may be used for the same film. The effective ratings for other types of film vary correspondingly.

After exposure, the film is developed, for example, for 13 minutes at 65° Fahrenheit in a 10 developer having preferably the following composition:

|                   |       |      |
|-------------------|-------|------|
| Metol             | grams | 4    |
| Sodium sulphite   | do    | 120  |
| Hydroquinone      | do    | 8.5  |
| Potassium alum    | do    | 40   |
| Potassium bromide | do    | 8    |
| Sodium hydroxide  | do    | 30   |
| Water             | cc    | 1000 |

20 It will be obvious that the composition of the developer may be varied considerably within the scope of the invention but there are a few features which must be kept substantially the same in such variation. The relation between the potassium alum and sodium hydroxide must remain practically constant, as described and claimed in my Patent No. 2,199,904, referred to above, and the proportion of sodium sulphite

25 must be kept high in order to effect the necessary solvent action on the silver salts in the emulsion. The potassium bromide may be varied considerably but the quantity suggested above is that which produces the least variation in the effect of the developer with use. The proportions and quantities of the Metol (or Elon) and hydroquinone may be varied considerably as is customary according to the type of contrast that is desired.

30 In the preparation of the developer the potassium alum will not completely dissolve until the sodium hydroxide is added. A gelatinous suspension is formed which is harmless but which may be filtered off, if desired. After the development the film should be rinsed in running water for about 30 seconds and then hardened in a hardening bath which may have the following composition:

|                  |       |      |
|------------------|-------|------|
| Sodium hydroxide | grams | 20   |
| Potassium alum   | do    | 26   |
| Paraformaldehyde | do    | 20   |
| Water            | cc    | 1000 |

35 After hardening for one or two minutes the film should be rinsed and then bleached in an

appropriate bleaching bath of which the following is typical:

|                            |            |      |
|----------------------------|------------|------|
| Potassium bichromate.....  | grams..... | 20   |
| Sulphuric acid concen..... | cc.....    | 20   |
| Water.....                 | do.....    | 1000 |

5

After the bleaching is complete the film should be rinsed and then cleared in a bath of 10 percent sodium sulphite in water.

After clearing the film should be washed thoroughly for at least 3 to 5 minutes in order to prevent any stain appearing during the second development. The film is then completely exposed and then developed in the second developer. This second developer may be the same as the first developer or it may be any ordinary type developer. One developer which is desirable for this purpose is that which is generally known as D 76, which produces a slightly finer grain structure in the final developed image than some of the other developers available.

The first developer which contains considerable alum prevents undue swelling of the emulsion during the development in spite of the large quantity of alkali used. Also, as described in my patent above referred to, the balance between the alum and alkali serves to stabilize the developer and prolongs its useful life to such an extent that it may be completely carried away by the film being processed before it is chemically exhausted.

The bleaching bath usually tends to produce considerable reticulation and this is prevented not only by the hardening developer but by the hardening bath suggested which, due to the combined action of the alum and paraformaldehyde, hardens the film to such an extent as to completely prevent any reticulation.

The degree of development suggested, together with the solvent action of the sodium sulphite, produces substantially clear whites which have been heretofore unattainable on this type of film and at the same time a proper gradation in the remainder of the image is produced.

Having now described my invention, I claim:

1. The reversal print producing method which

includes developing a silver halide emulsion in a developer containing balanced amounts of alum and alkali and a quantity of sodium sulphite approaching saturation, bleaching the film, exposing and redeveloping.

2. The method of producing reversal prints including the steps of developing a silver halide emulsion in a developer containing balanced amounts of alum and alkali and sodium sulphite approaching saturation, hardening the emulsion, bleaching the image, exposing and redeveloping.

3. The method of producing reversal silver halide emulsion prints comprising the steps of exposing a positive type film, developing the film in a developer containing balanced amounts of alum and alkali and a quantity of sodium sulphite approaching saturation, bleaching the film, exposing and redeveloping.

4. In the production of reversal silver halide emulsion photographic images, the step including the development of the original image in a developer containing balanced amounts of alum and sodium hydroxide and silver sulphite approaching saturation.

5. In the production of reversal silver halide emulsion photographic images, the step including the development of the original image in a developer containing balanced amounts of alum and sodium hydroxide and a quantity of sodium sulphite approaching saturation.

6. A photographic developer of silver halide emulsions including a developing agent, balanced amounts of alum and sodium hydroxide and a quantity of sodium sulphite approaching saturation.

7. A photographic developer having substantially the following composition:

|                        |            |      |
|------------------------|------------|------|
| Metol.....             | grams..... | 4    |
| Sodium sulphite.....   | do.....    | 120  |
| Hydroquinone.....      | do.....    | 8.5  |
| Potassium alum.....    | do.....    | 40   |
| Potassium bromide..... | do.....    | 8    |
| Sodium hydroxide.....  | do.....    | 30   |
| Water.....             | cc.....    | 1000 |

45

JAMES R. ALBURGER.